

May 22, 1928.

1,670,689

H. H. OLSTEAD

METHOD OF CASTING EXPLOSIVES

Filed Jan. 30, 1926

Fig. 1.



Fig. 2.



Fig. 3.



Fig. 4.



Inven. &  
Henry H. Olmstead

334 W. N. Roach.

Attorney

Patented May 22, 1928.

1,670,689

# UNITED STATES PATENT OFFICE.

HENRY H. OLSTEAD, OF WHARTON, NEW JERSEY.

## METHOD OF CASTING EXPLOSIVES.

Application filed January 30, 1926. Serial No. 85,027.

(GRANTED UNDER THE PROVISIONS OF THE ACT OF MARCH 3, 1883, 22 STAT. L. 625.)

The invention described herein may be used by the Government, or any of its officers or employees in prosecution of work for the Government, or by any other person 5 in the United States, without payment to me of any royalty thereon, in accordance with the act of March 3, 1883.

This invention relates to a cast of explosive and method of forming the same.

10 In order to secure the best results and maximum power in a bomb, mine, or the like, the explosive must be packed into the container or shell under a uniform high density.

15 The general procedure known as the "breaking-down" method which has been heretofore followed in loading bombs consists in pouring a rather large amount of molten explosive at a temperature of 79° C. 20 into the container, and after this has solidified to add gradually reduced increments. After each pouring a crust immediately forms upon the surface which retards the cooling of the semiliquid underneath. At 25 frequent intervals this crust is broken down and the liquid stirred. As the liquid cools and solidifies cavities are formed in the center of the mass so that before the final increments are added it is necessary to drill 30 holes in the center of the casts to reach all of the cavities. According to this method, several days are required to load a small bomb containing 150 lbs. of explosive.

The principal object, then, of this invention is to provide an improved method of loading containers such as bombs with an explosive charge of uniform and maximum density in a short period of time. I have discovered that it is impossible to cast explosives to a greater thickness than one-half inch without cavities and a layer of lower density forming between the upper and lower portions of the cast. To follow the above 40 rate of pouring in filling a container such as a bomb which is usually of a depth of from 5 to 7 feet would require an inordinately great period of time and I therefore propose in the present invention to provide a large number of casts each formed externally 45 of the container and comprising a laminated block, the layers of which are poured successively after stated cooling intervals and are of a thickness of approximately one-half inch.

50 To these and other ends, my invention con-

sists in the method of construction, described hereinafter and pointed out in the claims forming a part of this specification.

A practical embodiment of the invention is illustrated in the accompanying drawings, 60 wherein:

Fig. 1 is a longitudinal sectional view of a bomb loaded with casts formed according to the invention;

Fig. 2 is a vertical sectional view of one 65 of the casts;

Fig. 3 is a plan view thereof; and

Fig. 4 is an enlarged fragmentary sectional view through one of the staples provided for lowering the casts into the container. 70

Referring to the drawings by numerals of reference:

There is shown a bomb casing or shell 5 loaded with a plurality of laminated casts 75 6 of an explosive such as trinitrotoluene. The casts 6 may be of any desired thickness, preferably six inches, the controlling factors being convenience in loading and the relation of the cooling period to the usual working day.

The casts may be simultaneously formed in separate molds and the method of forming them consists in pouring, at intervals of thirty minutes, measured amounts of molten 80 explosive at a temperature of 79° C. into the mold forming layers 7—7, a half-inch in thickness. This allows a rapid cooling of the layers and insures uniform and maximum density without cavitation throughout 90 each layer. The cooling period of each layer is sufficiently short to permit twelve layers to be poured within the space of six hours so that one man tending to twenty-four molds every half hour would be able 95 during a working day to perform all tasks necessary to preparing the molds and removing the casts.

The casts are preferably formed with a convex bottom 8 and a concave top 9 100 to facilitate staking on loading them into the bomb and to insure centering.

Laminated casts formed according to my improved method possess considerable structural strength as it has been found in 105 breaking them with a hammer that the fragments break vertically to the layers and not on the line of division between the layers. However, if the casts are to be transported they may be strengthened by means of 110

metal rods 10 placed at any desired angle during formation of the casts.

If the bomb is to be loaded in a vertical position it is necessary to lower the casts 5 in place. To this end I may embed a pair of staples 11 in the cast while pouring the final increments. These staples are constricted as at 12 so as to be more firmly gripped and are embedded sufficiently deep 10 so as not to project above the concave upper face of the block. Any suitable apparatus may be provided for holding the staples when placing them into position. In lowering the cast into the bomb casing or raising it therefrom a rope or hook may be conveniently engaged with the staples. 15

This improved method of loading bombs possesses a great advantage over the "breaking-down" method in that the personnel are 20 exposed less to the absorption of the explosive.

I claim:

1. A method of forming casts of explosives which consists in pouring an amount of explosive into a mold to form a layer 25 approximately one-half inch in thickness, allowing it to cool for approximately thirty minutes, and successively adding and cooling increments of the explosive to form layers of similar thickness. 30

2. A method of forming casts of explosives which consists in pouring an amount of explosive into a mold to form a layer of approximately one-half inch in thickness, allowing it to cool, and successively adding 35 and cooling increments of the explosive to form layers of similar thickness.

3. A method of forming casts of explosives which consists in pouring an amount of explosive into a mold to form a thin layer, 40 allowing it to cool, and successively adding and cooling similar amounts of the explosive.

HENRY H. OLMSTEAD.